

## UNITED STATES PATENT OFFICE.

ALBERT SCHÖNHOLZER, OF HORN, SWITZERLAND, ASSIGNOR TO THE FIRM RADUNER & CO., A.-G., OF HORN (CT. THURGAU), SWITZERLAND.

## PROCESS FOR IMPARTING NEW EFFECTS TO COTTON FABRICS.

No Drawing.

Application filed February 11, 1924. Serial No. 692,172.

To all whom it may concern:

Be it known that I, ALBERT SCHÖNHOLZER, a citizen of the Republic of Switzerland, residing at Horn (Ct. Thurgau), Switzerland,

5 have invented certain new and useful Improvements in a Process for Imparting New Effects to Cotton Fabrics, of which the following is a specification.

It is already known to obtain transparent or wool-like effects on cotton fabrics or a linen-like lustrous appearance on fabrics having coarser yarns by the action of sulfuric acid of at least 50½° Bé. used at 10 normal temperature, i. e. above 5° C., and of sulfuric acid of below 50½° Bé. used at 15 temperatures below 0° C., and with or without a subsequent or preliminary treatment with alkali lye, and with or without being stretched, the effect obtained depending on 20 which of the various treatments is adopted.

The unexpected observation has now been made that if, instead of treating completely dry fabrics, as has been exclusively done up to the present, fabrics having a 25 content of moisture of at least 30% are subjected to the action of concentrated sulfuric acid of the above stated strengths, not a weaker alteration of the fabric is obtained as might be explained by the occurring dilution, but on the contrary much 30 more pronounced effects are obtained. The difference in the degree of action and in the alteration of the fabric thus caused is far greater than the difference presenting 35 itself by utilizing acid cooled to a low temperature as against using acid of a normal temperature.

This remarkable behaviour, which appears to be contradictory to the chemical 40 laws according to which the action must be intensified with increasing concentration, may be explained by assuming that in the present case the acid will penetrate much quicker and deeper into the interior 45 of the spun thread as well as of the fibre. As these differences in the effects are pronounced in the same manner whether the action of the acid is only very short or whether it lasts for several minutes, the 50 quicker penetration is not quite sufficient to explain the facts, the contents of water ap-

pear to operate to prepare the path for the acid and to place the material in condition to permit a deeper penetration of the acid than is the case with a dry fabric.

55 The technical utilization of this phenomenon renders it possible either to substantially reduce the acid concentration otherwise necessary or to shorten the time of action, which is of equal technical importance, in order to obtain the same effects as with the dry fabric and moreover to achieve novel effects with the moistened fabric consisting in substantially enhanced shrinking 60 effects.

65 Example 1.

Mercerized muslin fabric is uniformly moistened to a content of moisture of 80-100% and is then treated with sulphuric acid of a specific gravity of 1.535 equal to 50.8° Bé. at a temperature of 5° C. and for a period of 1 minute. The fabric obtained thereby has a full, wool-like appearance and a wool-like touch. A fabric which 70 for sake of comparison has been treated in the same manner with sulphuric acid, but which has not been moistened previous to the acid treatment is harder and dull and has no wool-like character.

75 Example 2.

Non-mercerized muslin fabric is moistened in the manner stated in example 1 and is thereupon treated with sulphuric acid of a specific gravity of 1.530 equal to 50° Bé. at 80 a temperature of 0° C. and for a period of 1 minute. Thereby a fabric having a very pronounced wool-like touch and which has shrunk very much is obtained; a fabric which has thus been treated without being 85 moistened shows much less shrinking.

90 Example 3.

Mercerized muslin fabric is moistened in the manner stated in example 1 and is then treated with sulphuric acid of a specific gravity of 1.530 to 1.535 at a temperature of 0° C. and for a period of 1 to 2 minutes. By means of a subsequent mercerizing under 95 tension with cold lye a good transparent effect is obtained and the fabric has an enhanced softness over transparent fabrics 100.

obtained when treating the dry fabric at lower temperatures or with acids of a higher concentration.

5 *Example 4.*

Upon mercerized or non-mercerized muslin fabric any desired pattern, for instance stripes, are printed immediately before the acid treatment by the aid of water so that 10 the printed parts are uniformly moist and are brought into the acid bath with a content of moisture of above 30%. If, for instance, acid of a specific gravity of 1.540 at a temperature of  $-10^{\circ}$  C. is used a very 15 pronounced pattern effect is obtained by this treatment as the threads become thicker and stick together. The obtained pattern effect may be enhanced by dyeing in consequence of the difference with which the 20 printed parts and the plain parts absorb the dye. Further the different action of the acid on these parts may be used to achieve crape effects.

The following effects obtained by the 25 treatment of moist fabrics and of dry fabrics may be stated for sake of comparison:

Mercerized muslin fabric:

1. Treatment with sulphuric acid of a 30 specific gravity of 1.520 at  $-10^{\circ}$  C. and for 1 minute:

The dry fabric is hardly changed, it gets somewhat coarser.

The moist fabric is completely changed it 35 is closer and becomes soft and wool-like.

2. Treatment with sulphuric acid of a specific gravity of 1.540 at  $-10^{\circ}$  C. and for 1 minute:

The dry fabric becomes transparent, hard 40 and coarse; the moist fabric becomes plastered up like paper.

Unmercerized muslin fabric:

3. Treatment with sulphuric acid of a specific gravity of 1.520 at  $-5^{\circ}$  C. and for 45 1 minute:

The dry fabric is made somewhat closer and becomes somewhat coarser.

The moist fabric is completely closed and an enhanced wool-like effect is obtained.

50 Instead of sulphuric acid other inorganic acids such as hydrochloric acid, nitric acid, phosphoric acid or a mixture of sulphuric acid and nitric acid in suitable effective concentrations may be employed. By means of 55 reserves the action of the acids or of the alkali solution may be prevented locally in order to produce pattern effects.

The present process may be applied to plain fabrics as well as to fabrics provided with patterns or embroideries.

60

I claim:

1. In the preparation of cotton fabrics for a treatment by acids for producing transparent or wool like effects, the step which comprises moistening at least part of the 65 fabric so that it contains moisture to an extent of not less than thirty per cent of the weight of the dry fabric so moistened and before subjecting it to the acid treatment.

2. In the preparation of mercerized cotton 70 fabrics for treatment by acids to produce transparent and wool-like effects, the step which comprises moistening at least part of the fabric so that it has a moisture content of at least thirty per cent of the dry fabric 75 that has been moistened and before the fabric is treated with acid.

3. In the preparation of cotton fabrics for treatment by acids to produce a transparent or wool-like effect, the step which 80 comprises moistening parts of a fabric to correspond to a desired pattern to an extent of at least thirty percent of the weight of that part of the dry fabric so moistened and before subjecting it to the acid treatment. 85

4. In the preparation of cotton fabrics for treatment by acids to produce a transparent or a wool like effect, the step which comprises printing a fabric with a reserve and providing a moisture content in the non- 90 printed portion of at least thirty percent of the weight of said non-printed portion when dry and previous to its immersion in the acid.

5. In the treatment of cotton fabrics by 95 such acids as are used to produce transparent or wool-like effects, the process which comprises moistening at least part of the fabric to an extent of not less than thirty percent of the weight of the dry fabric so 100 moistened previous to treatment with the acid, and after such treatment mercerizing the fabric.

6. In the treatment of cotton fabrics by such acids as are used to produce transparent 105 or wool-like effects, the process which comprises moistening at least part of a previously mercerized fabric with not less than thirty percent of the weight of the dry fabric so moistened, then subjecting it to the 110 action of the acid and subsequently mercerizing the acid treated fabric.

In testimony whereof I affix my signature.

ALBERT SCHÖNHOLZER.